

March 7, 1933.

P. J. MAUL ET AL

1,900,833

COATED CONCRETE

Filed Oct. 10, 1930

Fig. 1.



Fig. 2.



Fig. 3.



Fig. 4.



Inventors:  
Peter J. Maul,  
Martin Hoffman

By  
Ogunkiwa, Lee, Chittor & Wilcox  
Atggs:

## UNITED STATES PATENT OFFICE

PETER J. MAUL, OF DETROIT, MICHIGAN, AND MARTIN HOFFMAN, OF CHICAGO,  
ILLINOIS

## COATED CONCRETE

Application filed October 10, 1930. Serial No. 487,879.

This invention relates to coated concrete, and a method of producing it, and the primary object of the invention is to provide concrete having an improved waterproof 5 coating which, in some instances, is also employed for ornamental purposes.

The term "concrete" is employed generally to include concrete which is formed from cementitious material and various aggregates such as gravel, crushed stone, sand, cellular burned shale, cinders, granular cellular slag, etc.

Concrete embodying the invention is provided with a coating which is sprayed thereon in a fused state. In practicing the improved method, the coating material is reduced to a powder, and this powder is sprayed on the concrete in an oxy-acetylene flame, or the equivalent for the purpose. In 10 one embodiment of the invention, the powdered coating material is advanced to the oxy-acetylene flame in a tube of cellulose, lead, or any other suitable substance, and in another embodiment of the invention the powdered coating material is formed into a ribbon or strand by combining it with a binder. In the latter form, the ribbon or strand of powdered coating material is advanced into the flame which fuses the coating material and either fuses or burns up the binder.

In certain embodiments of the invention, coating or glazing material is incorporated in the concrete so that when the oxy-acetylene flame, or the equivalent, is directed thereon, the coating or glazing material on the surface of the concrete will fuse. Additional coating material is preferably sprayed upon the concrete through the oxy-acetylene flame and this combines with the coating material exposed on the surface of the concrete.

In the drawing:

Figure 1 is a perspective view, partly broken away, of a coated concrete block 45 which embodies the invention.

Fig. 2 is a somewhat diagrammatic section taken through an oxy-acetylene torch comprising means for spraying powdered coating material on concrete.

Fig. 3 is a perspective view of a tube filled 50 with powdered coating material, and

Fig. 4 is a perspective view of a strand of powdered coating material which is held in strand form by a binder.

In Fig. 1, a coated block of concrete embodying the invention is shown, the block being one of the type commonly employed in building construction, etc. It is to be understood, however, that the invention is not limited to this use as the invention may be employed in lighting posts, poles for telephone and power wires, shingles, roofing tile, roofing slabs, garden furniture, statuary, coffins, and in any other articles which are formed 55 from concrete.

The block shown in Fig. 1 comprises a body portion 10 and a coating 11. The body portion 10 may be made of cementitious material and any suitable aggregate such as gravel, crushed stone, sand, cinders, granular slag, or the like, but in the preferred embodiment of the invention cellular burned shale is employed as the main or principal aggregate. One form of cellular burned shale suitable for this purpose is known as 70 "Haydite" and this is preferably employed. The body portion 10 also comprises finely divided coating or glazing material for a purpose which will presently appear.

The coating 11 is formed by spraying coating material on the body portion 10. The coating material may comprise substantially any commercial glaze. Among the materials that may be employed are feldspar, alumina, lead and alkali glazes. One glaze which is 80 particularly suitable for the purpose comprises 258 parts by weight of white lead, 51.6 parts of Kaolin and 72 parts of flint, and another glaze particularly suitable for the purpose comprises 154.8 parts by weight of 85 90

white lead, 30 parts of calcium carbonate, 55.7 parts of feldspar, 25.8 parts of Kaolin and 48 parts of flint, these materials being in powder form.

5 Any suitable apparatus may be employed for spraying and fusing the powdered coating material, but the powdered material is preferably sprayed through an oxy-acetylene flame, or the equivalent. In Fig. 2, an 10 oxy-acetylene torch 15 is shown, which torch comprises a nozzle 16 and tubes 17 and 18 which communicate with sources of compressed oxygen and acetylene gas, respectively. The oxygen and acetylene gas are 15 mixed in a mixing chamber 19 and as the gaseous mixture passes to the nozzle 16 it draws the coating powder 20 from a receptacle 21 which is carried by the torch. The powder is drawn into the torch through a 20 tube 22 which projects from the receptacle 21. When the powdered material is sprayed onto the concrete, it fuses either in the flame or on the concrete, depending upon the temperature of the flame and upon the materials 25 from which the coating is made. Sufficient material is sprayed onto the concrete to give a coating of the desired thickness.

In another embodiment of the invention, the coating material, in powdered form, is 30 encased in a flexible tube. Thus, in Fig. 3, powdered coating material 25 is shown encased in a flexible tube 26 which has, preferably, a very thin wall. The tube 26 may be made of any suitable material, and among 35 the materials contemplated for this purpose are lead and cellulose. Thus, cellulose tubing formed from viscose extruded through an annular orifice and regenerated may be stuffed with the powdered coating material 40 and advanced into an oxy-acetylene flame to be sprayed thereby onto the concrete.

Another embodiment of the invention is illustrated in Fig. 4, wherein we have shown a strand 27 comprising powdered coating material mixed with a suitable binder. Binders employing such materials as glycerine, sodium silicate, litharge, and the like, are suitable for this purpose. The strand 27 may be advanced into an oxy-acetylene flame, or 50 the like, and sprayed thereby onto the concrete, the powdered coating material being fused either in the flame or upon the concrete.

As indicated above, coating material is preferably mixed with the aggregate and cementitious material forming the body portion 10. The coating material for this purpose preferably comprises powdered feldspar, ground glass, borax, or the like. The coating material constitutes about 10% of the concrete. 55 Then when the coating material is applied to the outer surfaces of the block by an oxy-acetylene flame, or the like, the coating material which is part of the concrete mixture and is exposed on the surfaces of the block, 60 fuses and combines with the powdered coat-

ing material which is projected onto the block by the oxy-acetylene flame. In practicing the improved method, the concrete is preferably preheated with an oxy-acetylene flame, or the equivalent, and, of course, such preheating also fuses the coating material exposed on the surface of the concrete.

70 In some embodiments of the invention, we contemplate employing finely divided metals, such as zinc, copper, brass, or the equivalent, 75 for forming the coating 11. The finely divided metals may be sprayed onto the concrete in the same manner as the powdered glazes described above, and it is to be understood that the appended claims should be construed to include the use of finely divided metals as coating material unless it is otherwise indicated.

80 As indicated above, the aggregate employed in the concrete is preferably "Haydite" which is a cellular burned shale. Cellular burned shale is light in weight and does not disintegrate or fuse when subjected to 85 relatively high temperatures, its fusing temperature being approximately 2100° F. In other embodiments of the invention, granular cellular slag from blast furnaces may be 90 employed. This cellular vitrified slag is discharged from the blast furnace at a temperature of about 3000° F. and is water cooled so that it becomes relatively cellular and light 95 in weight. One product of this character is sold under the trade name "Pottesco".

100 It is readily understood that the coatings embodying the invention may be made in various colors by employing suitable materials. Ornamental effects may be obtained in various ways. Thus, coatings of different colors may be applied to the same surface to 105 give a variegated effect.

110 While we have shown and described certain embodiments of our invention, it is to be understood that it is capable of many modifications. Changes, therefore, in the construction and arrangement may be made without departing from the spirit and scope of the invention as disclosed in the appended claims, in which it is our intention to claim 115 all novelty inherent in our invention as broadly as possible, in view of the prior art.

120 What we claim as new, and desire to secure by letters patent, is:

1. An article formed from concrete having a glaze on a surface thereof formed from glazing material mixed in the concrete.
2. An article formed from concrete having a glaze on a surface thereof formed from glazing material mixed in the concrete, and a coating on said glaze.
3. An article formed from cementitious material, cellular burned shale and a glazing material, said article having a glaze formed from the glazing material exposed on a surface thereof.
4. An article formed from cementitious

material, a cellular aggregate and a glazing material, said article having a glaze formed from the glazing material exposed on a surface thereof.

5 5. An article formed from cementitious material, a cellular aggregate and a glazing material, said article having a glaze formed from the glazing material exposed on a surface thereof, and a coating on said glaze.

10 In testimony whereof, we hereunto affix our names this 29th day of September, 1930.

PETER J. MAUL.  
MARTIN HOFFMAN.

15

20

25

30

35

40

45

50

55

60

65